

Jan. 27, 1931.

G. A. RICHTER

1,790,170

## PROCESS FOR THE PRODUCTION OF HIGH ALPHA CELLULOSE FIBER

Original Filed May 6, 1925



## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PROCESS FOR THE PRODUCTION OF HIGH ALPHA-CELLULOSE FIBER

Application filed May 6, 1925, Serial No. 26,339. Renewed July 23, 1927.

This invention relates to the utilization of the heat and the recovery of spent sodium digesting constituent from the spent liquor of an alpha-cellulose fiber plant operated 5 simultaneously or in connection with a kraft or "sodium sulphate" plant.

High alpha-cellulose fiber may be produced by an alkaline digestion of, for instance, unbleached sulphite pulp,—a caustic soda, soda 10 ash, or mixed caustic soda and soda ash solution being especially adapted for such digestion. The alkaline solution reacts with and dissolves the lignin and the less-resistant beta and gamma celluloses contained in the sulphite pulp, and after a sufficient period of 15 digestion yields a pulp which contains about 94% alpha or resistant cellulose, and has a very white color after bleaching. The alkaline digestion may take place in digesters at any suitable temperatures and pressures, 20 although I have found it in many cases to be more economical and expedient to digest the sulphite pulp at atmospheric pressure in open tanks under heat. In order to render the 25 process more economical, the spent sodium constituent should be recovered and the available heat content of the spent liquor should be utilized.

In my co-pending application Serial No. 26,361, filed April 28, 1925, a process for the recovery of the sodium constituent and the utilization of the available heat content of the spent digesting liquor has been outlined. Such a process, however, requires a special 35 recovery plant, where it is practiced in a plant wherein sulphite pulp only is produced. The object of this invention is to provide a method for practicing the economies set forth in the co-pending application, while combining the 40 recovery of sodium constituent from the spent liquor in an alpha-cellulose plant with the recovery of sodium constituent from the spent black liquor of a kraft plant, thereby eliminating the necessity for special recovery apparatus in the alpha-cellulose plant. This 45 invention may best be understood from the following description thereof, when taken in connection with the accompanying drawing, which represents what may be termed a flow 50 sheet.

Before proceeding to the features of invention involved herein, the operation of the alpha plant, which has been fully described in the co-pending application, will be briefly reviewed.

Sulphite pulp is produced, as usual, by the digestion of wood chips (e. g., spruce) in a digester, in a suitable sulphite liquor, as, for example, calcium bisulphite digesting liquor. After the necessary period of digestion, the 55 digester contents are blown, and the sulphite pulp is successively washed, screened, and thickened to, say, a consistency of about 50%, as by press rolls. The thickened, unbleached sulphite stock thus obtained is continuously 60 fed into a digesting tank A, and is diluted to a consistency of about 10% with water and the amount of caustic soda or soda ash solution required for the purification of the sulphite pulp. The diluted sulphite pulp is continuously 65 delivered into the bottom portion of a second digesting tank B, from the tank A, at the same rate as it is being made up in the tank A, by a slow-moving worm conveyor, and overflows from the second tank B. The 70 stock is digested and slowly agitated during its passage through the tanks A and B at 180° F. to 212° F., by blowing steam at suitable points into the suspension,—the less-resistant celluloses and the ligneous and other 75 coloring matters contained in the sulphite pulp reacting with and being dissolved by the alkaline solution so that the product which leaves the top portion of the second tank B is high in alpha or resistant cellulose. The agitation provided for during the digestion and the feed of the stock by the worm 80 from one tank to the other gives intimate contact between the stock and the liquor, and thereby promotes a thorough reaction between the sulphite pulp and the alkaline liquor, resulting in a uniform high alpha-cellulose pulp product. Of course, the digestion 85 may be carried out as a batch process, but obviously a continuous cyclic process is preferable.

The stock, together with the spent digesting liquor associated therewith, leaving the top portion of tank B, and now containing a high percentage of alpha-cellulose, is passed 90 95 100

through a counter-current washer, wherein the stock is thoroughly washed free from substantially all the digesting liquor, and the washed stock is then passed to the bleachery. The wash water used in the washing apparatus assumes practically the same temperature as the hot spent digesting liquor and the hot pulp as they are passed in the washing apparatus. The hot wash water (which for convenience of designation I term the "alpha spent liquor") contains substantially all the sodium constituent in any form, spent or otherwise, associated with the alpha stock as it was passed into the washer. The alpha spent liquor is re-circulated to the digesting tank A, and comprises in volume approximately the volume of water associated with the pulp after digestion, plus the total volume of wash water used in the washer, minus that portion absorbed by the washed alpha pulp as it passes to the bleachery. During this stage of the process, the volume of this wash water employed in washing the digested sulphite pulp is so regulated that the volume of spent alpha liquor obtained from the washer and re-circulated into the tank A is substantially equal to the volume of water and digesting solution employed in making up the initial 10% stock suspension in the tank A. To this re-circulated wash water is continuously added a sufficient quantity of 50% sulphite pulp and the amount of concentrated caustic soda or soda ash solution necessary to remove the less-resistant celluloses and the ligneous matter contained in the sulphite pulp to produce a stock suspension of about 10%. The new 10% stock suspension formed with the re-circulated wash water is digested, and the cycle of operations as hereinbefore described in connection with the initial 10% stock suspension is repeated. The hot spent liquor obtained from the washer at this point in the process contains a higher per cent of dissolved material. This spent liquor is recirculated as before and the process as described is continued or repeated until a hot, syrupy spent liquor of about 10° to 15° Baumé results. Such a concentrated spent liquor may profitably be evaporated and the combustible content thereof burned to recover the valuable sodium constituent. When this concentration of spent liquor is arrived at, the flow of fresh water to the washer is increased. As stated previously, up to this point the volume of spent liquor delivered from the washer has been only sufficient to dilute the incoming unbleached sulphite stock to a 10% consistency, or sufficient to ensure such consistency when the volume of solution containing fresh digesting constituent is taken into account; but there is now an excess of spent liquor. This excess is continuously withdrawn from the spent liquor obtained from the washer, and mixed with the black liquor resulting from a kraft

or sulphate pulp digestion as it is passed to the evaporators. The rest of the spent alpha liquor is re-circulated into the alpha digesting tank A. The increase in quantity of wash water,—that is, the excess passed along with the black liquor to the evaporators, is so adjusted as to maintain an equilibrium within the system at this particular concentration: that is, the excess spent liquor mixed with the spent kraft liquor contains substantially the amount of spent sodium constituent which was formed in the preceding digestion (the term "sodium" or "sodium constituent" as used in this specification and the appended claims will, of course, be understood to mean sodium in combined form, that is, in the form of a sodium compound). 70 80 90

As indicated on the drawing, it may be stated that the black spent liquor hereinbefore referred to results from the digestion of wood chips in a digester in the usual kraft or sulphate digesting liquor, which contains essentially caustic soda, sodium sulphide, together with a small quantity of sodium carbonate. After digestion, the digester contents are blown and the kraft pulp is passed through a counter-current washer similar to the one in which the alpha-cellulose pulp is washed. The wash water from the washer contains substantially all the digesting constituent associated with the kraft pulp as it is passed into the washer, is black and of about a 14° Baumé, and is known as spent kraft liquor. In some cases, it may be desirable to re-circulate one portion (usually about one-half the total of such spent liquor to the kraft digester) for use together with newly made digesting liquor in a subsequent kraft digestion. The other portion of black kraft spent liquor is passed into a storage tank, from which it is continually withdrawn to the evaporators. To this black liquor, as has been previously stated, is added the excess spent liquor of from 10° to 15° Baumé, obtained from the alpha spent liquor, so that a mixture of alpha and kraft liquors of about the same degree Baumé is passed into the evaporators for concentration. The resulting concentrate is burned, preferably in a combined boiler and smelting furnace, in a reducing atmosphere. Additional sulphur may be added as described in Letters Patent No. 1,469,960, dated October 9, 1923,—to the mixed concentrated liquor,—the amount of sulphur added thereto being regulated and controlled so as to form a smelt of approximately the same composition as the usual kraft smelt. The effluent smelt from the furnace is caught in a relatively small quantity of water in a dissolving tank, and a concentrated solution is formed which contains essentially sodium carbonate, sodium sulphide, and relatively small quantities of un-reduced sodium sulphate and sodium hydroxide. This solution is then causticized with lime, 100 110 120 130

in the usual manner, filtered, and the strong resultant white sulphide liquor, which contains sodium hydroxide, sodium sulphide, and smaller quantities of unreduced sulphate and unconverted sodium carbonate, is passed to a storage tank.

This strong white liquor may furnish a portion of the alkaline digesting agent required in the alpha plant tanks. This portion is preferably such that, together with the unspent alkali present in the re-circulated portion of spent alpha liquor, it contains the total alkali necessary for the alpha digestion, minus the losses suffered in both the alpha and kraft pulp cycles. From the foregoing statement it is obvious that if the alpha pulp and kraft pulp production happen to be in a certain proportion, that is, when the foregoing difference is zero or a minus quantity, no white liquor will be supplied to the alpha pulp digesters, in which case the alkali necessary for the alpha digestion is supplied directly to the digesting tank A, as shown. To understand this more clearly, the following example will suffice.

The sodium sulphate losses in a very efficient kraft plant amount to about 220 pounds of salt cake (sodium sulphate) per ton of pulp produced. The salt cake required to make up these losses is equivalent to about 125 pounds of caustic soda, and would represent the new caustic required to be added in the alpha digesters, when the make-up losses in the kraft mill are added only in the form of spent alpha liquor and sulphur. On the other hand, it so happens that about 125 pounds of caustic soda are required to treat a ton of unbleached sulphite pulp in the production of high alpha pulp. Assuming, then, that the alpha plant and the kraft plant are producing the same quantities of pulp, the spent liquor recovered from the alpha-cellulose plant delivered to the kraft plant contains just enough constituent to correspond to the losses in the kraft plant: that is to say, the total recovered sodium in the mixed spent liquors would contain just the correct amount of sodium constituent for the next digestion in the kraft plant, and under such conditions no white liquor would be delivered to the alpha digesting tanks. In other words, the recovered sodium constituent from a ton of alpha pulp would serve as a make-up material for the sodium losses suffered in producing a ton of kraft pulp, and in such a case it would be necessary to add to the alpha tanks the total sodium losses suffered in both cycles, which would be equal to the amount of sodium constituent required for digesting the unbleached sulphite pulp.

In actual practice, however, it is quite likely that such a balance could not be maintained, since the quantity of alpha pulp produced might be slightly in excess of the kraft pulp production, so that the white

liquor produced in the recovery of the digesting constituent from the mixed spent liquors would contain a certain amount of white liquor in excess of that required for the next kraft digestion, and this excess would be returned to the alpha digesting tanks. In addition to this returned white liquor, in order to maintain the system at equilibrium, an amount of alkali equal to the kraft and alpha cycle losses is added to the alpha digesting tanks, and the entire cycle may be repeated. Or, if the quantity of kraft pulp produced is slightly in excess of the alpha pulp production, no white liquor would be delivered to the alpha digesters. In this case, the amount of alkali which it would be necessary to introduce into the alpha digesters if the production of both the alpha and kraft plants were equal is then added to the alpha digesters. The kraft cycle losses not made up by the added spent alpha liquor to the recovery system are made up by the addition of sufficient sodium constituent in the form of sodium sulphate, or in the form of sodium carbonate, caustic soda, and sulphur, to the mixed spent liquor so as to give the usual kraft smelt.

Under conditions when no alkaline liquor is available from the kraft mill, then the unbleached sulphite pulp is digested entirely in caustic soda digesting liquor. If the alpha fiber plant uses available liquor from the kraft mill, there are present in the liquor a certain amount of sodium sulphide and a relatively small amount of other constituents, so that the sulphite pulp is digested in a mixture of caustic soda and sodium sulphide. Such a liquor produces as satisfactory an alpha pulp as is produced with caustic soda solution alone. Of course, the digesting liquor may be a solution of sodium carbonate or of a mixture of sodium carbonate and caustic soda, or of a mixture of sodium carbonate, sodium hydroxide, and sodium sulphide, or any other combination of these constituents.

Aside from the advantages outlined in the co-pending application, this invention provides for the recovery of sodium constituent and available heat content from the spent liquor in the alpha fiber plant, without the installation of special recovery apparatus.

I do not herein claim any features generic to application, Serial No. 72,522, filed December 1, 1925, by Milton O. Schur and myself; nor do I herein claim any features generic to my applications Serial Nos. 26,361 and 26,362, both filed April 28, 1925.

What I claim is:

1. A process which comprises digesting predigested pulp in an alkaline liquor containing sodium digesting constituent recovered from the spent liquor resulting from the digestion of cellulose material in the production of sulphate or kraft pulp, together

with the spent liquor resulting from previous digestion of like predigested pulp with alkaline liquor.

2. A process which comprises digesting predigested pulp in a fresh alkaline liquor containing sodium compounds, mixing sufficient spent liquor from such digestion with spent kraft liquor to make up sodium losses suffered in the kraft digesting cycle, and 10 recovering the sodium constituent from the spent mixed liquors.

3. An inter-related process of producing high alpha-cellulose pulp and kraft pulp, which comprises digesting predigested pulp 15 in an alkaline liquor containing sodium compounds, re-employing one portion of the spent liquor of the first-mentioned digestion in another digestion of like predigested pulp, and mixing the other portion with the spent 20 black liquor from kraft digestion, recovering the sodium constituent of the mixture, and using recovered sodium constituent in a subsequent kraft digestion and any excess thereof in another digestion of predigested pulp.

25 4. An inter-related process of producing high alpha-cellulose pulp and kraft pulp, which comprises digesting predigested pulp in an alkaline liquor containing sodium compounds, re-employing one portion of the 30 spent liquor of the first-mentioned digestion in another digestion of predigested pulp, mixing the other portion containing substantially the amount of spent digesting agent formed in a preceding digestion with 35 the black liquor resulting from kraft digestion, recovering the sodium constituent of the mixture, using the recovered sodium constituent necessary for the kraft digestion in such digestion, and using any excess recovered sodium constituent in another digestion 40 of predigested pulp, together with the re-employed portion of said first-mentioned spent liquor.

45 5. A process which comprises digesting predigested pulp in an alkaline liquor containing sodium compounds, mixing one portion of the spent digesting liquor with the black spent liquor resulting from a kraft digestion, recovering the sodium constituent 50 thereof, making up losses in the kraft cycle with the sodium constituent recovered from said one portion, re-employing the other portion of the spent liquor in another digestion of predigested pulp, adding any available 55 recovered sodium constituent to said other portion, and making up losses in both digesting cycles by the addition of sodium digesting agent to said other portion.

60 6. A process which comprises digesting predigested pulp in an alkaline liquor containing sodium compounds, re-employing one portion of the spent liquor in another digestion of predigested pulp, and mixing the other portion of the spent liquor containing 65 substantially the amount of spent digesting

agent which was formed in a preceding digestion with the black liquor resulting from a kraft digestion, recovering the sodium constituent thereof, and mixing a portion of said recovered constituent with the portion of re-employed spent liquor.

70 7. A process which comprises digesting predigested pulp in an alkaline liquor containing sodium compounds, re-employing substantially all the spent alkaline liquor of the digestion in another digestion of like pulp after the addition of sufficient sodium digesting agent thereto to make up losses therein for effective digestion, continuing such re-employment until a predetermined concentration of sodium results therein, and thereafter mixing one portion of the spent sodium alkaline liquor with the black liquor resulting from a kraft digestion, recovering the sodium constituents from the mixed liquor using the recovered sodium constituent in a subsequent kraft digestion, and re-employing the other portion of spent liquor in a subsequent digestion of predigested pulp.

75 8. A process which comprises digesting predigested pulp in an alkaline liquor containing sodium compounds, re-employing substantially all the spent alkaline liquor of the digestion in another pulp digestion after the addition of sufficient sodium digesting agent thereto to make up losses therein for effective digestion, continuing such re-employment until a predetermined concentration of sodium results therein, and thereafter re-employing one portion of the spent sodium alkaline liquor in another digestion of predigested pulp and mixing the other portion of the spent liquor with the black liquor resulting from a kraft digestion, recovering the sodium constituent from the mixed liquors, and using a portion of the recovered sodium constituent in a subsequent digestion of predigested pulp.

80 9. A process which comprises digesting predigested pulp in a fresh alkaline sodium base liquor, mixing spent liquor from such digestion with spent liquor resulting from the digestion of cellulosic material in kraft liquor, and recovering the sodium constituent from the spent mixed liquors.

85 10. A continuous cyclic process which comprises continuously feeding and digesting predigested pulp in an alkaline liquor containing sodium compounds, washing the resulting pulp and the entrained products of the reaction, circulating a part of the wash water back for further digestion of predigested pulp, mixing the other part with the black spent liquor resulting from a kraft digestion, evaporating said mixed liquor, burning and smelting the combustible content thereof in a reducing atmosphere, recovering the molten smelt in water, causticizing the resulting alkaline liquor, re-employing said 90

liquor in a subsequent kraft digestion, and employing any excess of said liquor in a subsequent digestion with said recirculated wash water in the digestion of predigested pulp, and making up losses in both digesting cycles by the addition of sodium compounds to said recirculated wash water.

11. Process comprising the following steps: digesting sulfite pulp in an alkaline liquor containing sodium sulfide to the formation of a pulp having a high alpha cellulose content and waste alkaline liquor and using this waste alkaline liquor in the preparation of a cooking liquor for a sulfate digestion of wood.

12. The process of making chemical wood pulp having a high content of alpha cellulose involving the digestion of raw cellulose material in an acid sulfite cooking liquor, separation of the resulting waste sulfite liquor from the resulting sulfite pulp, and digestion of the sulfite pulp in an alkaline cooking liquor, characterized in that the said alkaline cooking liquor is a solution comprising sodium sulfide obtained by concentrating smelting and recovering the sodium compounds present in the waste liquor from a collateral sulfate process of making pulp.

13. The process of making chemical wood pulp having a high content of alpha cellulose involving the digestion of raw cellulosic material in an acid sulfite cooking liquor, separation of the resulting waste sulfite liquor from the resulting sulfite pulp, and digestion of the sulfite pulp in an alkaline cooking liquor, characterized in that the said alkaline cooking liquor is a solution obtained by concentrating and smelting, in a reducing atmosphere, the waste liquor from a collateral sulfate process of making pulp, dissolving the resulting smelt in water, and treating the resulting solution with caustic lime.

In testimony whereof I have affixed my signature.

15

GEORGE A. RICHTER.

50

55

60

65